

## UNITED STATES PATENT OFFICE

2,115,374

COLORATION OF MATERIALS CONTAINING  
CELLULOSE ESTERS

James Arthur Wainwright and John Allan, Spon-  
don, near Derby, England, assignors to Celanese  
Corporation of America, a corporation of Del-  
aware

No Drawing. Application May 15, 1936, Serial  
No. 79,928. In Great Britain May 24, 1935

4 Claims.

(Cl. 8—5)

This invention relates to the production of ornamental effects on materials.

Various methods are employed for the production of pattern effects on textile materials. Thus, for example, a color may be applied directly to a material by printing and fixed thereon by steaming or other suitable after-treatment. Again, the material may be colored all over and then printed with a composition containing a discharging agent for the ground color so that the coloration is destroyed in the printed areas.

According to the present invention, pattern effects are produced on textile or other materials containing a cellulose ester by applying in a pattern a coloring matter or component having no affinity or small affinity for the cellulose ester and good affinity for cellulosic materials, before or after saponifying the cellulose ester in a pattern which coincides only in part with the pattern in which the coloring matter or component is applied. When a dye component is used it is subsequently converted into a dyestuff on the material.

By this process the coloring matter or component is fixed in parts only of the pattern in which it is applied, whereby a broken design is produced, or the design is in a deeper shade where the coloring matter pattern falls on a saponified area than where it falls on an unsaponified area.

For the local saponification of the cellulose ester, a saponifying agent (e. g. caustic soda) may be applied in suitably thickened preparations, which may contain swelling agents for the cellulose ester, and any other desired ingredients, by printing, stencilling, or other convenient method of local application, and the materials dried at elevated temperatures, and washed free from the saponifying agent. Instead of applying a saponifying agent locally to fabrics containing a cellulose ester, in order to produce locally saponified areas thereon, these areas may be obtained on the fabrics by employing intermittently saponified filaments or yarns in the construction of the fabrics.

Any convenient dyestuffs or dyestuff components having a good affinity for cellulosic materials and low affinity for cellulose esters under the conditions of application may be employed in the production of the pattern effects. Thus, for example, there may be employed direct cotton dyestuffs, chrome mordant printing colors, or azo dye components which may subsequently be coupled on the material to form the azo dyestuff, for example the sodium salts of enolic

coupling components, e. g.  $\beta$ -naphthol, 2:3-oxy-naphthoic arylamides, the diacylacetol derivatives of aromatic diamines, or pyrazolones. Because of the great fastness of the colorations obtainable with sulphuric and other esters of leuco vat dyestuffs, such for example as those sold under the trade name "Indigosol", it is preferred however to use these coloring matters for the formation of the colored patterns.

Thus, for example, pattern effects in very fast shades may be obtained in accordance with the present invention by applying an esterified leuco compound of a vat dyestuff in a pattern to a locally saponified cellulose ester material, so that only a part of the pattern falls on the saponified area, and developing the coloring matter without steaming. In many cases there is just sufficient fixation of the dyestuff on the cellulose ester for a shadow design to be obtained completing the broken design which appears where the coloring matter falls on a saponified area. Where the saponification process involves a heat treatment under moist conditions, it is advisable when working with these esterified leuco vat dyestuffs to apply the dyestuff composition to the locally saponified material rather than to saponify locally after applying the dyestuff.

A large variety of sulphuric and other esters of leuco vat dyestuffs, whether of the indigoid or anthraquinone series, may be employed in the process of the present invention. As examples there may be mentioned the following

| Dyestuff                            | See                                                           | 35 |
|-------------------------------------|---------------------------------------------------------------|----|
| Indigosol Yellow HCG powder         | Color Index No. 1176 and Supp. p. 16.                         |    |
| Indigosol Golden Yellow IGK powder  | G. Schultz, Farbstofftabellen, 7th Edition, 1st Supp. p. 108. |    |
| Indigosol Orange HR powder          | Color Index No. 1217, Supp. p. 17.                            |    |
| Indigosol Scarlet HB powder         | Color Index Supp. p. 43.                                      |    |
| Indigosol Pink IR powder            | G. Schultz, Farbstofftabellen, 7th Edition, 1st Supp. p. 109. |    |
| Indigosol Brilliant Pink 13B powder | G. Schultz, Farbstofftabellen, 7th Edition, 1st Supp. p. 108. |    |
| Indigosol Red HR powder             | Color Index Supp. p. 43.                                      |    |
| Indigosol Printing Blue IGG powder  | G. Schultz, Farbstofftabellen, 7th Edition, 1st Supp. p. 108. |    |
| Indigosol Printing Blue IB powder   | G. Schultz, Farbstofftabellen, 7th Edition, 1st Supp. p. 108. |    |
| Indigosol HB powder                 | Color Index Supp. p. 43.                                      |    |
| Indigosol O4B powder                | Color Index No. 1184, Supp. p. 16.                            |    |
| Indigosol Violet AZB powder         | Color Index, Supp. p. 43.                                     |    |
| Indigosol Green AB powder           | G. Schultz, Farbstofftabellen, 7th Edition, 1st Supp. p. 108  | 50 |

The coloring matter composition applied may contain any other desired ingredients in addition to the dyestuff or dye component. Thus, 55

for example, it may contain thickening agents, dyestuffs having affinity for cellulose esters and not for cellulosic materials, and assistants, such, for example, as diethylene glycol or thioglycol. 5 Further variations in design wherein a broken design is completed in another color may be obtained by incorporating in the printing compositions, dyestuffs having no affinity for cellulosic materials and good affinity for cellulose ester materials, and coloring the cellulose ester component in a shade different from that produced on the saponified material in accordance with the present invention.

Where esterified leuco vat dyestuffs are employed, agents adapted to give rise to oxidation of the dyestuff during a subsequent treatment may be incorporated in the composition to be applied. Especial mention is made of agents such, for example, as sodium nitrite or a chlorate, e. g. aluminium chloride, adapted to exercise their oxidizing action under acidic conditions. Where a chlorate or sodium nitrite is employed, a small quantity of ammonia or other alkali is preferably also incorporated in the composition to prevent premature oxidation of the leuco compound. The oxidation may be assisted by the presence of oxidation catalysts, e. g. copper salts or ammonium or other vanadate, which are conveniently applied to the material before the application of the esterified leuco compound. 25

Any convenient method of local application may be employed for the application of the coloring matter composition. Thus, the compositions may be applied by printing, whether screen printing or printing with engraved blocks or rollers, or by brushing or spraying through stencils. After application of the coloring matter or component the materials are subjected to suitable fixing or other treatments. For the development of an esterified leuco vat dyestuff applied in conjunction with a chlorate or nitrite, the treated materials are dried at low temperatures and developed in an acid bath, e. g. a mineral acid bath containing sulphuric acid, and then washed, soaped, and again washed and dried. The esterified leuco vat dyestuff will be removed from the cellulose ester portions of the materials but fixed on the saponified portions of the material. Where a direct cotton dyestuff is employed, a steaming or other fixing treatment may be applied, and the materials then washed to remove the dyestuff from the unsaponified material. 50

The effects produced in accordance with the present invention may be varied, for example by printing first with resist compositions so that the resist composition falls in part on an area wherein fixation of the coloring matter on saponified cellulose ester material would have occurred in the absence of the resist. For this purpose mechanical or other resists may be employed. For resisting esterified leuco vat dyestuffs a reducing agent, such, for example, as a hydrosulphite, may be applied locally to the materials, which will destroy or neutralize the oxidizing agent and prevent the development of the leuco vat dyestuff color in the selected areas. Other effects may be obtained if the fabric treated in accordance with the present invention is a mixed material, containing a cellulose ester and some other type of fibre. Thus, for example, the materials may contain alternate cellulose ester yarns and cellulosic and/or cellulose ether or natural silk yarns. 70

The following examples illustrate the invention without being in any way limitative. The 75 parts are by weight:—

### Example 1

A cellulose acetate woven fabric is printed in a bold design with the following saponifying composition:—

|                              | Parts | 5  |
|------------------------------|-------|----|
| Caustic soda                 | 15    |    |
| British gum thickening (1:1) | 50    |    |
| Glycerol                     | 5     |    |
| Water                        | 30    | 10 |

and is then dried, washed well with dilute acid, washed to free from acid, and again dried. The printed material is then over-printed in a small design with the following composition:—

|                                    | Parts | 15 |
|------------------------------------|-------|----|
| Indigosol Yellow HCG powder        | 6     |    |
| Indigosol Printing Blue IGG powder | 2     |    |
| Water                              | 41    |    |
| Thioglycol                         | 3     |    |
| Ammonia (10%)                      | 5     | 20 |
| Gum of tragacanth (8%)             | 40    |    |
| Sodium nitrite                     | 3     |    |

The printed material is dried and then developed in an aqueous solution containing 25 ccs. 25 per litre of 168° Tw. sulphuric acid at 60° C. and is then washed, soaped, washed again and dried.

A deep coloration occurs where the Indigosol print falls on the saponified area and a faint coloration where the Indigosol print falls on the 30 unsaponified areas of the fabric.

### Example 2

A woven fabric having a cellulose acetate weft and an intermittently saponified cellulose acetate warp is prepared with the following solution:— 35

|                   | Parts |    |
|-------------------|-------|----|
| Ammonium vanadate | 1     |    |
| Tartaric acid     | 5     |    |
| Water             | 94    | 40 |

and is then dried.

The treated material is then printed in a bold design with the following composition:—

|                              | Parts | 45 |
|------------------------------|-------|----|
| Golden Yellow IGK powder     | 6     |    |
| Water                        | 46    |    |
| Gum tragacanth (8%)          | 40    |    |
| Tartaric acid (10% solution) | 2.3   |    |
| Aluminium chlorate (42° Tw.) | 5     | 50 |

The printed material is then dried, hung in the air for about a day, and then well washed and dried.

Having described our invention what we desire to secure by Letters Patent is:— 55

1. Process for the production of pattern effects on textile materials containing cellulose acetate, which comprises saponifying the cellulose acetate in a pattern, then applying an esterified leuco vat dyestuff which has slight affinity for the cellulose acetate together with a nitrite in a pattern which coincides in part only with the pattern in which the saponification has been effected, and finally developing the coloring matter by treatment with an acid so that a shadow effect is obtained on the unsaponified portions of the material. 60

2. Process for the production of pattern effects on textile materials containing cellulose acetate, which comprises locally saponifying the cellulose acetate in a pattern, impregnating the material with a vanadate, and then applying an esterified leuco vat dyestuff which has slight affinity for the cellulose acetate in admixture with aluminium chlorate in a pattern which coincides in 70 75

part only with the pattern in which saponification has been effected, and allowing development of the coloring matter by the action of the chlorate to proceed so that a shadow effect is obtained on the unsaponified portions of the material.

5. 3. Process for the production of pattern effects on textile materials containing a cellulose ester, which comprises locally saponifying the cellulose ester and thereafter applying thereto an esterified leuco vat dye-stuff which has slight affinity for the cellulose ester in a pattern which coincides in part only with the pattern in which saponification has been effected and finally developing the coloring matter so that a shadow

effect is obtained on the unsaponified portions of the material.

4. Process for the production of a patterned textile fabric, which comprises applying to a cellulose acetate fabric containing in a pattern saponified cellulose acetate, a pattern in an esterified leuco vat dyestuff which has slight affinity for the cellulose acetate, so that the pattern of the coloring matter coincides in part only with the pattern of the saponified cellulose acetate, and then developing the coloring matter so that a shadow effect is obtained on the unsaponified portions of the material.

JAMES ARTHUR WAINWRIGHT.

JOHN ALLAN.

15